

## UNITED STATES PATENT OFFICE

2,385,496

## ZINC BASE ALLOY

Edward S. Bunn, Rome, N. Y., assignor to Revere  
Copper and Brass Incorporated, Rome, N. Y., a  
corporation of Maryland

No Drawing. Application June 10, 1943.  
Serial No. 490,327.

4 Claims. (CL 75—178)

My invention, which relates to zinc base alloys, and has among its objects the provision of a zinc base alloy of improved characteristics, will be best understood from the following description, the scope of the invention being more particularly pointed out in the appended claims.

The alloys according to the present invention consist of additions to zinc of 1 to 5% copper, 0.1 to 0.75% aluminum, and 0.03 to 0.5% silver, proportioned to each other as hereinafter specified.

It has been found that by adding to zinc small amounts of copper, aluminum and silver in proper proportions within the above specified ranges the zinc is given an exceedingly high tensile strength, the resulting alloy further having excellent hot working properties and resistance to impact loading or shock, coupled with freedom from intergranular corrosion and with satisfactory stability with age in respect to maintaining its tensile strength, resistance to shock, and dimensions. Although the ductility of the alloy is not as high as that of some zinc base alloys, it nevertheless is sufficiently high to be satisfactory for many uses, particularly where an alloy is required for fabricating by hot working an article of high unit strength.

The improved alloys it is believed have tensile strengths superior to any high content zinc base alloy yet produced. In this respect the alloys with low amounts of alloying contents are comparable to high tensile strength forging brass, and with high amounts of alloying contents are much superior to forging brass and are comparable to aluminum bronze. For example, the alloy with 5% copper, 0.75% aluminum, and as little as 0.1% silver has a tensile strength of about 68,000 pounds per square inch. If the amount of aluminum in this alloy is reduced to 0.1% the alloy will still have a very high tensile strength of 60,000 pounds per square inch, and even if the amount of copper is reduced to 1% will still have a very high tensile strength of 57,000 pounds per square inch. Even with as little as 1% copper, 0.1% aluminum and 0.1% silver the alloy still has a tensile strength of 40,000 pounds per square inch.

It has been found that the addition of aluminum to zinc, although much increasing its tensile strength, tends to reduce its ductility to a very unsatisfactory extent and to cause, as the resulting binary alloy ages, intercrystalline corrosion, and, further, sufficient formation of an additional alloy phase to make it unstable in respect to dimensions, thus making the alloy un-

satisfactory in all these respects. These defects imparted by the aluminum it has been found cannot be satisfactorily eliminated by adding copper with the aluminum. However, it has been found that the combination of silver and copper when added to the zinc with the aluminum, within the ranges and proportions herein specified, has the remarkable effect of compensating for these defects tended to be imparted by the aluminum in that it effectively prevents intercrystalline corrosion, alloy phase change and dimensional instability, and improves the ductility in the unaged, annealed and aged conditions sufficiently to make the resulting alloy satisfactory in that respect for many uses. Further, the addition of silver acts very markedly to increase the resistance of the alloy to shock and impact loading as compared to pure zinc or zinc which has aluminum alone or both copper and aluminum added to it, and therefore in that respect further increases the usefulness of the alloy.

Although best suited for hot working by rolling, forging, etc., the improved alloys are still sufficiently ductile in the cold condition for light stamping and drawing operations. They however find their greatest field of usefulness where stable alloys of very high tensile strength and resistance to shock are required for making hot forged articles.

Within the ranges of constituents herein specified the above properties of the alloy will be secured provided the sum of the amounts of silver and aluminum does not substantially exceed the amount of copper, and, when the amount of copper is 1.5% or less, the amount of silver does not substantially exceed the amount of aluminum. If the sum of the amounts of silver and aluminum present in the zinc substantially exceeds the amount of copper present the resulting alloy will be unsatisfactorily deficient in respect to ductility, and may be subject to intergranular corrosion and dimensional instability as the alloy ages. If the amount of copper is approximately 1.5% or less, and the amount of silver present substantially exceeds the amount of aluminum present, the alloy further will be deficient in tensile strength and lack satisfactory stability in that respect as the alloy ages. In respect to the amount of silver added, best results will be secured when the silver is within the range of 0.07 to 0.25%. The tensile strength of the alloy increases with the amounts of copper or aluminum added, and the ductility decreases with these amounts. Best results in respect to tensile

strength are secured when at least 0.3% aluminum and 3% copper are present. When the aluminum is not over 0.4%, and the copper not over 2.5%, best results will be secured in respect to ductility.

It will be understood that, within the scope of the appended claims, further constituents may be added for modifying the properties of the alloy or securing additional properties, so long as the characteristic properties imparted by the addition of copper, aluminum and silver to the zinc are not substantially destroyed.

I claim:

1. Zinc base alloys having, approximately, 1 to 5% copper, 0.1 to 0.75% aluminum, 0.03 to 0.5% silver, the sum of the percentage amounts of aluminum and silver not substantially exceeding the percentage amount of copper, and, for amounts of copper up to 1.5%, the percentage amount of silver not substantially exceeding the

percentage amount of aluminum, the balance being substantially zinc.

2. Zinc base alloys having, approximately, 1 to 5% copper, 0.1 to 0.75% aluminum, and 0.07 to 0.25% silver, the percentage amount of silver not substantially exceeding the percentage amount of aluminum when the amount of copper is substantially less than 1.5%, the balance being substantially zinc.

3. Zinc base alloys having, approximately, 1 to 2.5% copper, 0.1 to 0.4% aluminum, 0.07 to 0.4% silver, the percentage amount of silver not substantially exceeding the percentage amount of aluminum when the amount of copper is substantially less than 1.5%, the balance being substantially zinc.

4. Zinc base alloys having, approximately, 3 to 5% copper, 0.3 to 0.75% aluminum, 0.07 to 0.5% silver, the balance being substantially zinc.

EDWARD S. BUNN.